

June 6, 1950

J. W. PEDLOW ET AL

2,510,135

METHOD FOR SPINNING ARTIFICIAL FILAMENTS

Filed Aug. 25, 1947



INVENTOR.  
JOHN WATSON PEDLOW  
WESLEY L. WEBB  
INGHAM S. ROBERTS

By *Thomas R. McVay*

## UNITED STATES PATENT OFFICE

2,510,135

## METHOD FOR SPINNING ARTIFICIAL FILAMENTS

John Watson Pedlow, Chester Heights, Wesley L. Webb, Glen Moore, and Ingham S. Roberts, Ridley Park, Pa., assignors to American Viscose Corporation, Wilmington, Del., a corporation of Delaware

Application August 25, 1947, Serial No. 770,372

20 Claims. (Cl. 18—54)

1

This invention relates to methods of spinning artificial filaments by the wet-spinning system in accordance with which filaments extruded through orifices of a spinneret enter a coagulating liquid which serves to set up the filaments either by removal of solvent or by chemical reaction therewith.

In the past, there have been many attempts to control the flow of the coagulating liquid relative to the filaments issuing from the spinneret in order to produce artificial filaments having better qualities, and particularly uniformity of strength, extensibility, and dyeing throughout the length of each filament and also among the several filaments issuing not only from a single spinneret but from all of the spinnerets in a given machine. However, the spinning procedures heretofore employed allow the filaments to be subjected to variable stresses by the coagulating liquid before the filaments were toughened by sufficient setting or coagulation to be insensitive to such variable influences so that the final physical properties of the filaments were non-uniform, and this non-uniformity existed along the length of each individual filament as well as between the several filaments issuing from the same or different spinnerets. In general, therefore, such attempts have only been partially successful.

It has now been discovered that it is possible to produce in a practical manner artificial filaments which are markedly improved in respect to strengths, both wet and dry, extensibilities, wet and dry, and dyeing, particularly in respect to the uniformity of such characteristics among the several filaments issuing from a single spinneret as well as along the length of each filament and even among the filaments issuing from several spinnerets, by an improved manner of controlling the action of the coagulating liquid upon the freshly extruded filaments.

In general, the new process involves forcing a small stream or jet of the coagulating liquid to move midair along with the freshly extruded filament bundle through a straight path at substantially the same speed as the filaments while avoiding irregular disturbances resulting from part of the liquid running back upon or ahead of, or dripping off, the traveling filament-liquid stream until such stream reaches a predetermined stage at which removal of the liquid can be accomplished in a uniform manner and under conditions subject to control.

It has been found that a small but substantial quantity of liquid will adhere as a body to the filaments so that substantially all of such liquid

2

will travel with the filaments and at the same velocity as the filaments over considerable distances through the air without any noticeable change of velocity regardless of the direction of the flight through the air. The amount of liquid that can thus adhere to the filament bundle and be sustained and moved along bodily with it, in spite of gravitational and air friction forces depends on a number of factors including the particular filament-forming material, the number of filaments making up the bundle, and the nature of the coagulating liquid, particularly its surface tension, viscosity and tendency to adhere to the material constituting the filaments. The maximum amount that can thus travel with the filaments is not inconsiderable, however, and it has been found that, in general, much less than the maximum permissible amount will in a relatively short passage even at spinning speeds higher than conventional, set up the filament-forming streams of material to a sufficiently firm condition that the filaments leaving this stage of production can stand up under all the customary subsequent treating stages without being unduly sensitive to irregularities therein.

In order to limit the amount of liquid traveling with the thread, the spinneret may be disposed within a chamber to which the coagulating liquid is supplied, which chamber is provided with an opening in front of the spinneret face through which the filaments accompanied by the liquid are withdrawn. This opening may be of sufficiently small diameter to limit the amount of liquid passing out of the chamber with the filaments; depending upon the nature of the material forming the opening and the precise contour at the opening, the diameter of the stream issuing may increase or decrease somewhat from the diameter of the opening and accordingly the selection of the size of the opening should take this into account. The chamber about the spinneret should be kept filled with the coagulating liquid which involves the feeding of such liquid thereto at a rate sufficient to equal the rate of withdrawal by the filaments. In the vicinity of the opening, the contour of walls about the passage or zone within the chamber is preferably streamlined to assure viscous flow of the liquid as it approaches the opening immediately before passage therethrough. This can be adequately met by gradually tapering the inside wall or walls of the chamber toward the opening.

The accompanying drawing is illustrative of the spinning processes of the present invention.

Figure 1 is an axial section through a spinneret

assembly which may be used in performing the invention,

Figure 2 is an elevation showing one spinning system,

Figure 3 illustrates a modification,

Figure 4 is a plan view of the embodiment of Figure 3, and

Figure 5 is illustrative of a modification in which spinning is performed in a downward direction.

As illustrated in Figure 1, each spinneret is advantageously disposed within an individual chamber to which the coagulating liquid is supplied, though it is to be understood several spinnerets may be disposed in a common chamber. In Figure 1, the spinneret 3 is held in place upon a supply pipe 4 by means of the coupling 5, a gasket 6 being present to provide a seal. A housing member 7 is held in place upon the coupling member 5 by means of the sleeve 8 which threadedly engages the outer periphery of coupling 5. The member 7 contains the chamber 9 and has a recess 10 within which a guiding element 11 having an orifice 11b fits. A gasket 12 is seated between the member 11 and the shoulder at the back of the recess 10 and the orificed member 11 is held in place by a coupling sleeve 13 which threadedly engages the outer periphery of the housing member 7.

The coagulating liquid is supplied to the chamber 9 by means of the conduit 14 which may be the discharge conduit of a metering pump 15 such as a gear pump. The conduit 14 fits into the housing member 7 and is arranged to direct the coagulating liquid around the body of the spinneret 3.

As shown, it is preferable, when spinning certain materials into certain baths which develop gases during the spinning such as viscose into an acid regenerating bath, to have a portion or even all of the coagulating liquid stream discharged by the conduit 14 directed across the face 3a of the spinneret in order to prevent accumulation of bubbles on the spinneret face. The arrows generally indicate the flow of the coagulating liquid around the spinneret and then into the region immediately in front of the spinneret face. The inner end wall of the member 11 projects inwardly of the adjacent inside wall of the housing and this projecting ledge or shoulder assures that the liquid flows from all sides of the outer periphery of the spinneret toward the center of its face. As the liquid flows inwardly along the face, it contacts with the filaments leaving the several orifices within the spinneret, sweeps gas bubbles from the face, and joins with the filaments in the main current of flow axially of the spinneret and of the tapered bore 11a in the guiding member 11. The transverse flow of the coagulating liquid over the face of the spinneret, though shown as proceeding from all points of the spinneret face periphery, may proceed from one side only of such face so that the transverse flow may deflect the filament-forming streams toward the other side of the spinneret face, as is shown in the copending patent application of Roberts Serial No. 698,437, filed September 21, 1946. This sweeping of the spinneret face is unnecessary, however, when spinning other materials or under conditions which do not develop gas bubbles.

The size of the opening 11b may be preselected, as more particularly described hereinafter, to limit the diameter of the stream or jet of liquid traveling with the filaments from the spinneret

assembly. The guide element or nozzle 11 is preferably made of material which is not only resistant to corrosion, erosion, and abrasion, but exerts but little abrading action on any filaments that may occasionally rub thereagainst during the initial lacing or threading operations. Glass, porcelain, agate, lava, and artificial materials of the latter type, such as that available under the trade name "Alsimag" may be used to advantage for this fitting. The tapered passage 11a merging into the opening 11b may have any length up to 10 cm. or so but is preferably relatively short so that the distance from the opening 11b back to the spinneret face is not over 2 or 3 cm.

15 As illustrated in Figures 2 to 5, the spinneret assembly may be arranged to discharge the liquid carrying the filament bundle in any direction from vertically downward to vertically upward. Regardless of the direction taken by the filaments during spinning, i. e., downwardly or upwardly or at an inclination to either direction, the control of the coagulating liquid supplied to the chamber may be accomplished either by means of a metering pump such as a gear pump or by the maintenance of a predetermined pressure upon the liquid supplied to the chamber. When dependence is placed upon a predetermined pressure rather than upon a metering pump, it then becomes more important to predetermine 30 the diameter of the opening 11b in order to limit the amount of liquid issuing with the filament bundle. Regardless of which system is employed for controlling the supply of coagulating liquid to the chamber, it is of paramount importance to 35 keep the chamber full of coagulating liquid at all times during spinning and also to provide a gradual taper along the bore 11a approaching the opening 11b. This taper assures substantially viscous flow of the coagulating medium 40 through the guiding member 11 and into the free flight or course through the air. Some turbulence may be present in the vicinity around the face of the spinneret where the coagulating liquid sweeps transversely of the filaments and then 45 must change direction to flow through the member 11, but is preferably minimized by forming the parts, such as the member 11 and the spinneret body, with smoothly rounded contours. Whatever small amount of turbulence there may 50 be at any part of the passage followed by the coagulating liquid through the chamber, the fact that the liquid is continuously supplied at a constant rate assures substantially uniform treatment of the filaments within such chamber.

55 The present invention, however, is more vitally concerned with what occurs after the filament-containing coagulating liquid stream or jet leaves the spinneret assembly up to the time of the removal of the excess liquid from the filament bundle. If the liquid carried by the filament 60 bundle begins to flow back down the bundle in the case of upward spinning, irregularities immediately occur which influence the properties of the filaments. Thus, as the liquid starts to 65 flow back down the liquid-carrying filament stream, it disturbs the upward traveling body of liquid and in a fashion characteristic of liquid, a more or less irregular wave pattern is generally set up by such disturbance. The result of 70 such a disturbance is inherently the production of an irregular filament. Such irregularity in the filament may not always be detectable in terms of its diameter but it does show up in variations of strength, extensibility and dye receptivity along the filament. Similarly, in down-

ward spinning, the overtaking mass of liquid similarly sets up a disturbance having a wave pattern of irregular character which again influences the filaments irregularly. When the direction of spinning is horizontal, upward or downward at an inclination to the vertical, part of the liquid may drip off the course of the filaments at irregularly varying distances from the spinneret assembly.

All of these irregular occurrences are avoided in accordance with the present invention by limiting the amount of liquid in the jet accompanying the filament bundle to the amount which is able to cohere as a unit and to adhere bodily to the given filament bundle throughout the free flight in midair in the particular direction at which spinning occurs without the back flow, overtaking, or dripping so that the liquid at any point along the bundle as it travels from the spinneret assembly has substantially the same linear velocity throughout its cross section as the filaments traveling therein. It is a relatively simple matter to determine when all of the liquid travels at the same speed as the filaments since, when this condition is present, the diameter of the stream remains constant from a point near the exit opening of the spinneret assembly all the way to the surface which removes the liquid from the filaments. The amount of liquid that can be carried in this fashion depends upon the particular nature of the spinning material and the coagulating liquid, but in general, it has been determined that a safe upper limit of load is 0.001 gram per centimeter per filament for bundles containing up to about 300 filaments and optimum results are obtained if the load per filament is not over 0.0006 gram per centimeter. The latter limit is applicable to bundles having any number of filaments such as 1200. In the spinning of viscose in a dilute acid aqueous coagulating bath having a specific gravity of 1.3 to 1.4, it has been found that the limit of load is reached when the filament-containing liquid stream has a diameter of 3 mm. and optimum results are obtained if the diameter does not exceed 2 mm.

The amount of liquid in the jet containing the filaments may be controlled in various ways. The size of the opening 11b can be predetermined to limit the diameter of the liquid jet issuing and the velocity of the jet can be controlled by pre-selecting the pressure exerted upon the liquid in the chamber 9, or by the operation of the metering pump, depending upon which device is employed. When operated in this fashion, the size of opening may vary in a practical fashion between about 0.5 mm. to 3.0 mm. in diameter though lesser diameters not exceeding 2 mm. are preferred.

When spinning upwardly, some reliance may be placed upon the natural tendency of the filament bundle to carry the liquid with it out of the opening, in which event the diameter of the opening can be much larger than and even several times the above-mentioned 3 mm. limit, but this is satisfactory only when the distance from the face of the spinneret to the liquid level in the exit opening in the chamber is not over 3 cm. and is preferably 2 cm. or less. The filament-containing jet of liquid issuing in this case acquires its velocity from the filaments being withdrawn from the assembly. The filament bundle itself, in this case, can be used to control the diameter of the liquid stream, and this can be effectively done by varying the spacing between the orifices of the spinneret. When wide spac-

ing, such as 0.020 to 0.040 inch between centers of adjacent orifices in a row and between centers of adjacent rows, is used, a relatively larger diameter of liquid stream will move away with the filaments, whereas a closer spacing, such as 0.005 to 0.015 inch between centers of adjacent orifices in a row and between centers of adjacent rows, provides a smaller diameter, and as indicated above, the smaller diameter streams are preferred. The closer spacing becomes more advantageous as the number of filaments in the bundle becomes larger.

In accordance with the present invention, it is desirable to remove the liquid in a controlled manner and this is preferably done by contacting the filament-containing stream with a surface having a linear speed substantially the same as that of the filaments. Such surface may be inclined to one side of the running filaments so that the liquid runs down the surface away from the filaments as they bear against the surface. Or, the surface may be a porous one so that the liquid flows to the interior thereof. Alternatively a rotary drum having a linear peripheral speed the same as that of the filaments may be lightly pressed against the straight course of the filaments before they reach the thread-advancing device, such as 16 in Figure 2, and the liquid removed by the surface may be wiped off the drum at a point away from that in contact with the filaments. Again, the surface may rotate at a sufficiently high speed (though still the same linear speed as that of the filaments) to throw the liquid off the filament bundle by centrifugal force as the filament bundle travels around such surface.

Figure 2 is illustrative of the present invention in which spinning is performed in a vertical and upward direction. As shown, the filaments extruded through the orifices of spinneret 3 within the chamber in housing 7 which is supplied with coagulating liquid by the conduit 14 leave the opening 11b in a stream of liquid traveling therewith at substantially the same speed. The filaments pass directly along a straight path from the opening 11b to a thread-advancing device such as the godet 16 having an inclined axis and about which the filaments are lapped by means of a roller guide 17. The godet 16 is driven at any desired spinning speed from 75 meters upwardly and in accordance with the present invention it has been found that spinning speeds as high as 200 meters per minute can be employed with satisfactory production of filaments. When the filaments first reach the peripheral surface of godet 16, they are pressed thereagainst and the liquid travels down to the rim 18 of the godet from which it may flow into a gutter 19 therebelow. Since all of the liquid carried with the filaments travels at the same speed throughout the passage from the spinneret to the godet 16, and the godet 16 removes the liquid uniformly from each point of the filament bundle as such points reach the surface in succession, there is no opportunity for the flow of liquid back down the filaments and the irregular disturbances developed thereby.

From the godet 16, the bundle of filaments from which the liquid has been removed, may pass to a second thread-advancing device which may comprise a godet 20 and associated wrap-displacing guide roller 21. Between the godets 16 and 20, the filaments may be stretched or allowed to relax in a fashion which is conventional in the art. From the godet 20, the filaments may pro-

ceed to additional thread-advancing devices to receive additional stretch or to allow shrinkage after one or two stages of stretching, or the filaments may proceed to other thread-advancing devices upon which they may be treated with liquids, such as for washing, bleaching, desulfurizing, decoppering, and the like. Whether or not the filaments leaving the godet 20 pass over additional thread-advancing devices for after-treatment, further stretching and the like, the filaments are ultimately collected either in the form of an untwisted or twisted package. For example, they may be collected in a centrifugal pot in the fashion conventional in the viscose spinning process; or they may be collected by winding on a bobbin without twisting; or they may be collected on twisters of the cap, flyer, or ring type.

The process of the present invention is particularly adaptable to continuous spinning processes and especially to such processes as require high speed spinning, such as that disclosed in the application of Stanley and Lowe, Serial No. 504,664, filed October 2, 1943. In this latter type of process, the filament proceeding from the spinning stage of the continuous spinning machine passes to one or more thread-advancing devices which rotate at sufficient speed to throw the liquid off by centrifugal force and a jacket is provided about the thread-advancing reel with its inner surface closely spaced about the bars of the reel so as to deflect the liquid thrown out to the surface back to the helix of filaments carried by the reel.

Figures 3 and 4 show a modification in which the filaments leaving the opening 11b in the housing 7 around the spinneret 3 pass upwardly at an inclination to the vertical and in this embodiment, the filaments in the jet of the coagulating liquid proceed directly to a thread-advancing reel 22 rotating at sufficiently high speed to throw the liquid from the helix of thread carried thereon. As shown more particularly in Figure 4 a guard member 23 is provided around the zone of the reel to which the filaments are first led. This guard member receives the liquid thrown off by centrifugal force and discharges it through a drain 24 connected to the bottom thereof. Beyond this zone of the reel, a jacket 25 is disposed entirely surrounding the reel and having an inside deflecting surface 26. Annular grooves 27 and 28 are disposed at each side of the surface 26 and communicate with drain pipes 29. Additional coagulating liquid may be supplied to this jacket by means of the pipe 30 communicating with the bore 31 into the surface 26. This

ring course between the spinneret assembly and the first thread-advancing device before subsequent washing, desulfurizing, etc., can be performed on a continuous spinning machine.

The coagulating liquid supplied to the jacket 25 is repeatedly thrown off the helix of filaments and deflected back thereon to provide a thorough washing in the manner disclosed in the above mentioned Stanley and Lowe application. From this reel, the filaments may proceed to a second reel operating at higher peripheral speed to effect stretching. A liquid may be applied to the filaments as they pass between the reels to facilitate stretching, such as hot water in the case of viscose. Then the filaments may proceed either to a collecting device or over a plurality of liquid-treating reels before being collected.

Figure 5 illustrates the directing of the filaments downwardly in a substantially vertical direction from the opening 11b of the housing 7 about the spinneret 3. The coagulating liquid supplied to the chamber within the housing 7 by the conduit 14 is metered by the opening 11b so that a limited weight of liquid travels with the filaments to the thread-advancing device 32. In this embodiment, the distance between the opening 11b and the point of first contact with the thread-advancing device 32 is preferably sufficient to provide substantially complete setting up of the filaments so that when they make contact with the device 32, they are no longer deleteriously affected by any accumulations of liquid on the device 32 with which they may make contact. However, the distance between the spinneret assembly and the device 32 may be less than that just specified, in which event it is desirable to incline the device 32 in the manner of device 18 in Figure 2, or to operate it at high peripheral speed as in Figure 3, in order to throw the liquid off by centrifugal force.

While the invention is applicable to the spinning of filaments of any material by the wet spinning procedure, the following examples illustrate the invention with reference to the spinning of viscose. These examples make use of a viscose containing 7½% cellulose and 6½% sodium hydroxide spun at a common salt point of 4, into a coagulating bath containing 9 to 10.5% sulfuric acid, 3% zinc, and 20 to 22% sodium sulfate at a temperature averaging 55° C. and having a specific gravity averaging about 1.38. The tabulated examples indicate the conditions which provide the travel of the coagulating liquid with the filaments at the same speed without back flow, dripping or overtaking.

| Ex.     | Total Denier | No. of Filaments | Dia. of 11b | Spinn. Speed | Rate of Bath Feed | Dia. of Liquid Fil. Jet | Bath wt. on Yarn |
|---------|--------------|------------------|-------------|--------------|-------------------|-------------------------|------------------|
|         |              |                  | Mm.         | M./min.      | cc./min.          | Mm.                     | g./cm.           |
| 1.....  | 150          | 40               | 2.0         | 100          | 290               | 2.0                     | 0.040            |
| 2.....  | 150          | 60               | 1.5         | 75           | 140               | 1.4                     | 0.026            |
| 3.....  | 150          | 60               | 1.5         | 100          | 165               | 1.5                     | 0.023            |
| 4.....  | 150          | 60               | 1.5         | 125          | 185               | 1.45                    | 0.020            |
| 5.....  | 150          | 60               | 1.5         | 150          | 210               | 1.4                     | 0.020            |
| 6.....  | 150          | 40               | 1.2         | 112.5        | 125               | 1.2                     | 0.015            |
| 7.....  | 150          | 60               | 1.5         | 112.5        | 210               | 1.6                     | 0.026            |
| 8.....  | 150          | 90               | 1.7         | 112.5        | 250               | 1.75                    | 0.031            |
| 9.....  | 250          | 120              | 1.8         | 112.5        | 300               | 1.9                     | 0.037            |
| 10..... | 1,100        | 490              | 2.7         | 112.5        | 710               | 2.9                     | 0.087            |
| 11..... | 150          | 60               | 1.0         | 97.5         | 90                | 1.0                     | 0.011            |
| 12..... | 50           | 24               | 1.5         | 200          | 300               | 1.4                     | 0.021            |
| 13..... | 75           | 30               | 0.9         | 97.5         | 60                | 0.7                     | 0.009            |
| 14..... | 100          | 40               | 1.5         | 175          | 300               | 1.45                    | 0.020            |

is particularly desirable in the case of spinning a viscose solution which generally takes additional contact with the coagulating liquid beyond that which could be effected in a single run-

The present invention not only controls the flow of coagulating liquid so that the amount carried by the filaments is not so excessive as to develop back flow and dripping and like irregular

disturbances but it also economizes on the amount of coagulating liquid needed for complete set up. Furthermore, it assures that the coagulating liquid which makes contact with the filaments immediately after the material leaves the spinneret orifices has a definite composition which is constant throughout the period of spinning. Thus, each portion of the length of each filament is in contact with a coagulating bath having a definite constitution at any point of its passage between the spinneret orifice and the stage at which coagulating liquid is removed. Fresh coagulating liquid of the predetermined constitution makes the first contact with the filaments issuing from the spinneret and such liquid, contaminated as a result of contact with the filaments, is not allowed to tarry at the spinneret face to react with subsequently issuing filaments but instead is continuously withdrawn with the filaments so that fresh liquid replaces that at the spinneret face in a continuous fashion. This action is assured by the provision of the relatively small chamber about the spinneret which is kept filled with coagulating liquid and is rapidly withdrawn with the filaments. Since the coagulating liquid always has a velocity in the direction of flow of the filaments from the spinneret face, there is very little of what may be termed a "bath drag" exerting any substantial tension upon the filaments as they pass from the spinneret to the stage at which the coagulating liquid is removed. In addition, the direct travel of the filaments from the spinneret face to the stage at which the liquid is removed in a controlled and uniform fashion assures that the characteristics of the filaments are as uniform as possible. The present invention is particularly advantageous in high speed spinning and for this purpose, its preferred form makes use of controlled pressure or a metering pump for delivering the coagulating liquid to the chamber about the spinneret at a predetermined rate, in combination with the preselection of the diameter of the opening in the chamber through which the filaments are discharged for controlling the diameter of the stream issued therefrom so that in effect, the liquid discharged from that opening serves to carry the filaments rather than the converse. When operating in this fashion, a high speed jet of liquid issues and assists the withdrawing device in carrying the filaments thereto.

It is to be understood that changes and variations may be made without departing from the spirit and scope of the invention as defined in the appended claims.

We claim:

1. The method of producing artificial filaments comprising continuously extruding a filament-forming material through the orifices of a spinneret into a stream of coagulating liquid flowing in the general direction of extrusion, directing the filament-forming streams of material in a straight path as they proceed from the spinneret and are coagulated to filaments in the coagulating liquid stream, imparting a predetermined constant velocity to the filaments as they proceed in said straight path, forming the coagulating liquid stream at a point within a distance of about 10 centimeters in front of the spinneret into a jet having substantially the same velocity as the filaments and flowing in free flight through the air along the straight path of the filaments, controlling the amount of liquid in the jet to assure that all of the liquid adheres to and travels substantially at the same velocity as the

filaments throughout said straight path, and then continuously removing liquid from the filaments in a uniformly controlled manner at a predetermined point of the straight path.

- 5 2. The method of claim 1 in which the direction of extrusion is upward.
3. The method of claim 1 in which the direction of extrusion is downward.
4. The method of claim 1 in which the direction of extrusion is vertically upward.
- 10 5. The method of claim 1 in which the direction of extrusion is vertically downward.
6. The method of producing artificial filaments comprising continuously extruding a filament-forming material through the orifices of a spinneret into a stream of coagulating liquid flowing at gradually increasing velocity in the general direction of extrusion; directing the filament-forming streams of material in a straight path as they proceed from the spinneret and are coagulated to filaments in the coagulating liquid stream; imparting a predetermined constant velocity to the filaments along said straight path; forming the coagulating liquid stream at a point within a 15 distance of about 10 centimeters in front of the spinneret into a jet having substantially the same velocity as the filaments, flowing in free flight through the air along the straight path of the filaments, and having a weight per centimeter of length not over 0.001 gram per filament so as to assure that all of the liquid adheres to and travels substantially at the same velocity as the filaments throughout said straight path, and then continuously removing liquid from 20 the filaments in a uniformly controlled manner at a predetermined point of the straight path.
- 25 7. The method of claim 6 in which the jet has a diameter not over 3 mm.
8. The method of claim 6 in which the jet has a diameter not over 2 mm.
9. The method of claim 6 in which the jet has a weight per centimeter of length not over 0.0006 gram per filament and a diameter not over 3 mm.
10. The method of claim 6 in which the jet has a weight per centimeter of length not over 0.0006 gram per filament and a diameter not over 2 mm.
11. The method of producing artificial filaments comprising continuously extruding a filament-forming material through the orifices of a spinneret into a stream of coagulating liquid, moving the liquid in said stream away from the spinneret at gradually increasing velocity in the general direction of extrusion, withdrawing the filament-forming streams of material from the spinneret in a straight path at a predetermined constant velocity, forming the coagulating liquid stream at a point within a distance of about 10 centimeters in front of the spinneret into a jet 40 having substantially the same velocity as the filaments and flowing in free flight through the air along the straight path of the filaments, controlling the amount of liquid in the jet to assure that all of the liquid adheres to and travels substantially at the same velocity as the filaments throughout said straight path, and then continuously removing liquid from the filaments in a uniformly controlled manner at a predetermined point of the straight path.
12. The method of claim 11 in which the jet has a weight per centimeter of length not over 0.001 gram per filament and a diameter not over 3 mm.
13. The method of claim 11 in which the jet has a weight per centimeter of length not over 0.0006

gram per filament and a diameter not over 2 mm.

14. The method of producing artificial filaments comprising continuously extruding a filament-forming material through the orifices of a spinneret into a confined passage not over about 10 centimeters in length and having a restricted exit opening, continuously directing coagulating liquid of predetermined constitution through the passage and the opening at sufficient velocity to form a jet of the liquid issuing from the opening, continuously withdrawing the filaments through the opening and directing them with the jet in a straight free flight at substantially the same speed as the jet, controlling the amount of liquid in the jet to assure that all of the liquid adheres to and travels substantially at the same velocity as the filaments throughout the free flight, and then continuously removing liquid from the filaments at the end of the free flight.

15. The method of claim 14 in which the jet has a weight per centimeter of length not over 0.001 gram per filament and a diameter not over 3 mm.

16. The method of claim 14 in which the jet has a weight per centimeter of length not over 0.0006 gram per filament and a diameter not over 2 mm.

17. The method of producing artificial filaments comprising continuously extruding a filament-forming material through the orifices of a spinneret into a confined passage having a restricted exit opening not over about 10 centimeters from the spinneret face and a transverse cross-section along a portion thereof decreasing gradually to, and merging with, the opening, continuously directing coagulating liquid of predetermined constitution through the passage and the opening at sufficient velocity to form a jet of the liquid issuing from the opening, continuously withdrawing the filaments through the opening and directing them with the jet in a straight free flight at substantially the same speed as the jet, controlling the amount of liquid in the jet to assure that all of the liquid adheres to and travels substantially at the same velocity as the filaments throughout the free flight, and then continuously removing liquid from the filaments at the end of the free flight.

18. The method of producing artificial filaments comprising continuously extruding a viscose spinning solution through the orifices of a spinneret into a confined passage having a restricted exit opening not over about 10 centimeters from the spinneret face and a transverse cross-section along a portion thereof, decreasing gradually to, and merging with, the opening, continuously directing an aqueous, acid coagulating liquid transversely past the viscose streams at the position of extrusion and then through the passage and the opening at sufficient velocity to form a jet of the liquid issuing from the opening, continuously withdrawing the filaments through the opening and directing them with the jet in a straight free flight at substantially the same speed as the jet, controlling the amount of liquid in the jet to assure that all of the liquid adheres to and travels substantially at

the same velocity as the filaments throughout the free flight, and then continuously removing liquid from the filaments at the end of the free flight.

19. The method of producing artificial filaments comprising continuously extruding a viscose spinning solution through the orifices of a spinneret, continuously directing an aqueous, acid coagulating liquid transversely past the viscose streams at the position of extrusion into a zone surrounding the viscose streams, directing the filaments from the vicinity of the spinneret along a straight path comprising beyond a distance not over about 10 centimeters from the spinneret face, a free flight portion proceeding at a predetermined constant velocity, passing all of the coagulating liquid contaminated by proximity to and contact with the viscose streams with gradually increasing velocity through said zone away from the spinneret in the same direction as the viscose streams while supporting the filaments thereby until the velocity of the liquid is approximately the same as that of the filaments, controlling the amount of liquid in contact with the filaments along the free flight portion to assure that all of the liquid adheres to and travels substantially at the same velocity as the filaments throughout said portion, and then continuously removing liquid from the filaments at the end of the free flight portion.

20. The method of producing artificial filaments comprising continuously extruding a filament-forming material through the orifices of a spinneret into a stream of coagulating liquid flowing in the general direction of extrusion, directing the filament-forming streams of material in a straight path as they proceed from the spinneret and are coagulated to filaments in the coagulating liquid stream, imparting a predetermined constant velocity to the filaments as they proceed in said straight path, forming the coagulating liquid stream at a point within a distance of 3 centimeters in front of the spinneret into a jet having substantially the same velocity as the filaments and flowing in free flight through the air along the straight path of the filaments, controlling the amount of liquid in the jet to assure that all of the liquid adheres to and travels substantially at the same velocity as the filaments throughout said straight path, and then continuously removing liquid from the filaments in a uniformly controlled manner at a predetermined point of the straight path.

JOHN WATSON PEDLOW.  
WESLEY L. WEBB.  
INGHAM S. ROBERTS.

#### REFERENCES CITED

The following references are of record in the file of this patent:

#### UNITED STATES PATENTS

Number Name Date  
1,493,545 Holken, Jr. May 13, 1924

#### FOREIGN PATENTS

Number Country Date  
65 394,049 Great Britain June 22, 1933